

## UNITED STATES PATENT OFFICE.

PAUL RABE, OF LEVERKUSEN, NEAR COLOGNE, AND WILHELM SCHEPSS, OF WIERSDORF, NEAR COLOGNE, GERMANY, ASSIGNEES, BY MESNE ASSIGNMENTS, TO GRASSELLI DYESTUFF CORPORATION, OF NEW YORK, N. Y., A CORPORATION OF DELAWARE.

## PROCESS FOR DYEING ACIDYL CELLULOSES.

No Drawing. Application filed March 3, 1924, Serial No. 696,675, and in Germany May 28, 1923.

It is well known that acidyl celluloses have only a small absorptive power for dyestuffs. Attempts have, therefore, not been lacking to avoid this defect. A process is described, for instance, in German Patent No. 355,533, which allows of the direct dyeing of cellulose acetate silk, by the addition to the dye-bath of one or more protective colloids, organic acids, and larger quantities of water-soluble salts, particularly chlorides. British Patent 179,384 also recommends the employment of metallic salts such as sodium stannate, magenta etc., with the simultaneous addition of colloids. The noteworthy fact has now been established, that salts of the oxy-acids of nitrogen and chlorine, as for instance, nitrates, chlorates, nitrites etc. are suitable in quite a peculiar degree, as additions in dyeing acidyl cellulose e. g., cellulose acetate silk, films etc. or their transformation products. The use of protective colloids is superfluous. Even relatively small quantities of these salts produce shades of hitherto unattainable depth. Example 1.—1 part by weight of chrysoidine G extra is dissolved in 1000 parts by weight of water and 5 parts by weight of aniline nitrate are added. Ratio 1:20. Dyeing temperature 70°. Time 30 minutes. Instead of aniline nitrate, the nitrates of ammonium, sodium, magnesium, calcium or zinc and further, of such organic bases as monomethylamine, dimethylamine etc., guanidine, pyridine and piperidine, may be used. Example 2.—1 part by weight of crystal

violet P is dissolved in 1000 parts by weight of water, and 5 parts by weight of sodium nitrite are added. Dyeing is performed as under 1. Chlorates may also be used instead of nitrates.

Other dyestuffs or their salts, as for instance, methylene blue, rhodulin red B, safranine, auramine, Bismark brown, rhodulin yellow, rhodulin blue 6G (nitrate), turquoise blue G, rhodamin 6G extra, new methylene blue F, and many others can be fixed on acetate cellulose silks in this manner, with extraordinary depth of shade.

Our application Ser. No. 755,037 filed December 10, 1924, contains subject matter divided out of this application.

We claim:—

1. Process of dyeing acidyl celluloses characterized in and by the fact that the acidyl celluloses are dyed in a bath containing a dye and a salt of an oxy acid of nitrogen.
2. Process of dyeing acidyl celluloses characterized in and by the fact that the acidyl celluloses are dyed in a bath containing aniline nitrate.
3. A dyeing composition comprising a dye and a salt of an oxy acid of nitrogen with an organic base.
4. A dyeing composition comprising a dye and aniline nitrate.

In testimony whereof we have hereunto set our hands.

PAUL RABE.  
WILHELM SCHEPSS.